

# United States Patent Office.

SIMON L. MADGE, OF TOLEDO, OHIO.

*Letters Patent No. 98,874, dated January 18, 1870.*

## IMPROVED METALLIC ALLOY FOR PLOW-MOULD-BOARDS.

The Schedule referred to in these Letters Patent and making part of the same.

To all whom it may concern:

Be it known that I, SIMON L. MADGE, of Toledo, in the county of Lucas, and State of Ohio, have invented a new and useful Improvement in Metallic Composition for Plows; and I do declare that the following is a true and accurate description thereof.

The nature of this invention relates to the combination of several metals, all of them cheap in cost, and common in the market, to be employed more especially in the manufacture of plows; and consists in the mixture made of the materials, and in the proportions, as more fully hereinafter described.

The various kinds of soil to be found in the United States, seem to require that plows shall be made of different materials, so that they will operate successfully in the different soils. For instance, in a soft muck soil, a steel plow is found to operate better than a cast-iron one, and the latter will work well in dry or sandy soils.

The design of this invention is to produce a metal for the manufacture of mould-boards, and landsides, and other similar articles, which will clean and keep smooth in all kinds of soils.

In order to accomplish this end, I melt pig-iron, and

when in a molten state, and ready for pouring into the flasks or moulds, I add to it tin and antimony, in the following proportions, to wit:

To a pound of cast-iron, I add one ounce of antimony, and one-half an ounce of tin. These, thoroughly incorporated together, and cast in the ordinary manner, will produce a casting that will have the appearance, when broken, of both sides being chilled, while the centre will present the appearance of a very fine-grained iron.

The effect, as well as appearance, is the same as though the iron had been cast in a chill, leaving the outer surfaces very fine-grained and hard, and susceptible of a high polish, like that of steel, without its liability to rust.

What I claim as my invention, and desire to secure by Letters Patent, is—

The alloy, when made of the metals, and substantially in the proportions and for the purposes herein described.

SIMON L. MADGE.

Witnesses:

JAS. I. DAY,  
R. C. SMITH.